



US005136761A

**United States Patent** [19]

Sternlieb et al.

[11] **Patent Number:** **5,136,761**[45] **Date of Patent:** **Aug. 11, 1992**[54] **APPARATUS AND METHOD FOR HYDROENHANCING FABRIC**

[75] Inventors: **Herschel Sternlieb**, Brunswick, Me.; **Jodie M. Siegel**, Somerville, Mass.; **John M. Greenway**, Westwood, Mass.; **Zoltan Mate**, Sherborn, Mass.; **Frank E. Malaney**, Milton, Mass.

[73] Assignee: **International Paper Company**, Purchase, N.Y.

[21] Appl. No.: **608,933**

[22] Filed: **Nov. 5, 1990**

|           |         |                  |         |
|-----------|---------|------------------|---------|
| 4,146,663 | 3/1979  | Ikeda et al.     | 428/96  |
| 4,156,957 | 6/1979  | McKay            | 28/159  |
| 4,190,695 | 2/1980  | Niederhauser     | 428/234 |
| 4,223,349 | 11/1980 | Niederhauser     | 428/92  |
| 4,251,587 | 2/1981  | Mimura et al.    | 428/233 |
| 4,329,763 | 5/1982  | Alexander et al. | 28/104  |
| 4,426,421 | 1/1984  | Nakamae et al.   | 428/234 |
| 4,497,095 | 2/1985  | Minemura et al.  | 26/2 R  |
| 4,499,637 | 2/1985  | Greenway         | 26/2 R  |
| 4,612,237 | 9/1986  | Frankenburg      | 428/219 |
| 4,695,500 | 9/1987  | Dyer et al.      | 428/134 |
| 4,808,467 | 2/1989  | Suskind et al.   | 428/284 |
| 5,037,692 | 8/1991  | Miyazaki et al.  | 428/252 |
| 5,047,276 | 9/1991  | Chomarat et al.  | 428/110 |

**Related U.S. Application Data**

[63] Continuation-in-part of Ser. No. 382,160, May 18, 1989, Pat. No. 4,967,456, and a continuation-in-part of Ser. No. 184,350, Apr. 21, 1988, abandoned, and a continuation-in-part of Ser. No. 41,542, Apr. 23, 1987, abandoned.

[51] Int. Cl.<sup>5</sup> ..... **D04H 1/46**  
[52] U.S. Cl. ..... **28/104; 8/151.2;**

**28/167; 68/205 R; 428/225**

[58] Field of Search ..... **28/104, 167; 8/151.2; 68/205 R; 428/225**

[56] **References Cited****U.S. PATENT DOCUMENTS**

|           |         |                   |         |
|-----------|---------|-------------------|---------|
| 2,241,222 | 5/1941  | Sonnino           | 26/2    |
| 3,214,819 | 11/1965 | Guerin            | 28/72.2 |
| 3,422,510 | 1/1969  | Livingston et al. | 28/1    |
| 3,485,706 | 12/1969 | Evans             | 161/72  |
| 3,498,874 | 3/1970  | Evans et al.      | 161/109 |
| 3,542,632 | 11/1970 | Eickhoff          | 161/65  |
| 3,873,255 | 3/1975  | Kalwaites         | 425/83  |
| 3,906,130 | 9/1975  | Tsurumi et al.    | 428/131 |
| 3,917,785 | 11/1975 | Kalwaites         | 264/108 |
| 4,144,370 | 3/1979  | Boulton           | 428/233 |
| 4,145,468 | 3/1979  | Mizoguchi et al.  | 428/239 |

**FOREIGN PATENT DOCUMENTS**

|          |        |                    |
|----------|--------|--------------------|
| 287821   | 9/1964 | Australia          |
| 739652   | 8/1966 | Canada             |
| 0177277  | 9/1985 | European Pat. Off. |
| 7410272  | 3/1974 | France             |
| 61-55253 | 3/1986 | Japan              |

*Primary Examiner*—Philip R. Coe*Attorney, Agent, or Firm*—Walt Thomas Zielinski[57] **ABSTRACT**

An apparatus **10** and related process for enhancement of woven and knit fabrics through use of dynamic fluids which entangle and bloom fabric yarns. A two stage enhancement process is employed in which top and bottom sides of the fabric are respectively supported on members **22, 34** and impacted with a fluid curtain including high pressure jet streams. Controlled process energies and use of support members **22, 34** having open areas **26, 36** which are aligned in offset relation to the process line produces fabrics having a uniform finish and improved characteristics including, edge fray, drape, stability, abrasion resistance, fabric weight and thickness.

26 Claims, 22 Drawing Sheets

10



—  
—  
—  
—  
—



FIG. 2A



FIG. 2B



FIG. 3A



FIG. 3B



FIG. 4A



FIG. 4B



FIG. 5A



FIG. 5B



FIG. 6 A



FIG. 6 B



FIG. 7A



FIG. 7B



FIG. 8A



FIG. 8B



FIG. 9A



FIG. 9B



FIG. 10A



FIG. 10B



**FIG. II A**



**FIG. II B**



FIG. 12A



FIG. 12B



FIG. 13A



FIG. 13B



FIG. 14A



FIG. 14B



FIG. 15A



FIG. 15B



FIG. 15C



**FIG. 16A**



**FIG. 16B**



FIG. 17A



FIG. 17B



**FIG. 18A**



**FIG. 18B**



FIG. 19



FIG. 20

**FIG. 2IA****FIG. 2IB**

## APPARATUS AND METHOD FOR HYDROENHANCING FABRIC

### CROSS REFERENCE TO RELATED APPLICATIONS

This application is a continuation-in-part of U.S. Ser. No. 07/382,160, filed May 18, 1989, now U.S. Pat No. 4,967,456, which was in turn a continuation-in-part of U.S. Ser. No. 07/184,350, filed Apr. 21, 1988, now abandoned, which was in turn a continuation-in-part of U.S. Ser. No. 07/041,542, filed Apr. 23, 1987, now abandoned.

### FIELD OF INVENTION

This invention generally relates to a textile finishing process for upgrading the quality of woven and knit fabrics. More particularly, it is concerned with a hydro-entangling process which enhances woven and knit fabrics through use of dynamic fluid jets to entangle and cause fabric yarns to bloom. Fabrics produced by the method of the invention have enhanced surface finish and durability and improved characteristics such as cover, abrasion resistance, drape, stability as well as reduced air permeability, wrinkle recovery, absorption, adsorption, shrink resistance, seam slippage, and edge fray.

### BACKGROUND ART

The quality of a woven or knit fabric can be measured by various properties, such as, the yarn count, thread count, abrasion resistance, cover, weight, yarn bulk, yarn bloom, torque resistance, wrinkle recovery, drape and hand.

Yarn count is the numerical designation given to indicate yarn size and is the relationship of length to weight.

Thread count in woven or knit fabrics, respectively, defines the number ends and picks, and wales and courses per inch of fabric. For example, the count of cloth is indicated by enumerating first the number of warp ends per inch, then the number of filling picks per inch. Thus, 68×72 defines a fabric having 68 warp ends and 72 filling picks per inch.

Abrasion resistance is the ability of a fabric to withstand loss of appearance, utility, pile or surface through destructive action of surface wear and rubbing.

Absorption is the process of gases or liquids being taken up into the pores of a fiber, yarn, or fabric.

Adsorption is the attraction of gases, liquids, or solids to surface areas of textile fibers, yarns, fabrics or any material.

Cover is the degree to which underlying structure in a fabric is concealed by surface material. A measure of cover is provided by fabric air permeability, that is, the ease with which air passes through the fabric. Permeability measures fundamental fabric qualities and characteristics such as filtration and cover.

Yarn bloom is a measure of the opening and spread of fibers in yarn.

Fabric weight is measured in weight per unit area, for example, the number of ounces per square yard.

Torque of fabric refers to that characteristic which tends to make it turn on itself as a result of twisting. It is desirable to remove or diminish torque in fabrics. For example, fabrics used in vertical blinds should have no

torque, since such torque will make the fabric twist when hanging in a strip.

Wrinkle recovery is the property of a fabric which enables it to recover from folding deformations.

5 Fabric surface durability is the resistance of a material to loss of physical properties or appearance as result of wear or dynamic operation.

Hand refers to tactile fabric properties such as softness and drapability.

10 It is known in the prior art to employ hydroentangling processes in the production of nonwoven materials. In conventional hydroentangling processes, webs of nonwoven fibers are treated with high pressure fluids while supported on apertured patterning screens. Typically,

15 the patterning screen is provided on a drum or continuous planar conveyor which traverses pressurized fluid jets to entangle the web into cohesive ordered fiber groups and configurations corresponding to open areas in the screen. Entanglement is effected by action of the fluid jets which cause fibers in the web to migrate to open areas in the screen, entangle and intertwine.

20 Prior art hydroentangling processes for producing patterned nonwoven fabrics are represented by U.S. Pat. Nos. 3,485,706 and 3,498,874, respectively, to Evans and Evans et al., and U.S. Pat. Nos. 3,873,255 and 3,917,785 to Kalwaites.

25 Hydroentangling technology has also been employed by the art to enhance woven and knit fabrics. In such applications warp and pick fibers in fabrics are hydroentangled at crossover points to effect enhancement in fabric cover. However, conventional processes have not proved entirely satisfactory in yielding uniform fabric enhancement. The art has also failed to develop apparatus and process line technology which achieves 30 production line efficiencies.

35 Australian Patent Specification 287821 to Bunting et al. is representative of the state of the art. Bunting impacts high speed columnar fluid streams on fabrics supported on coarse porous members. Preferred parameters employed in the Bunting process, described in the Specification Example Nos. XV-XVII, include 20 and 30 mesh support screens, fluid pressure of 1500 psi, and jet orifices having 0.007 inch diameters on 0.050 inch centers. Fabrics are processed employing multiple hydroentangling passes in which the fabric is reoriented on a bias direction with respect to the process direction in order to effect uniform entanglement. Data set forth in the Examples evidences a modest enhancement in fabric cover and stability.

40 Another approach of art is represented by European Patent Application 0 177 277 to Willbanks which is directed to hydropatterning technology. Willbanks impinges high velocity fluids onto woven, knitted and bonded fabrics for decorative effects. Patterning is effected by redistributing yarn tension within the fabric—yarns are selectively compacted, loosened and opened—to impart relief structure to the fabric.

45 Fabric enhancement of limited extent is obtained in Willbanks as a secondary product of the patterning process. However, Willbanks fails to suggest or teach a hydroentangling process that can be employed to uniformly enhance fabric characteristics. See Willbanks Example 4, page 40.

50 There is a need in the art for an improved woven textile hydroenhancing process which is commercially viable. It will be appreciated that fabric enhancement offers aesthetic and functional advantages which have application in a wide diversity of fabrics. Hydroen-

hancement improves fabric cover through dynamic fluid entanglement and bulking of fabric yarns for improved fabric stability. These results are advantageously obtained without requirement of conventional fabric finishing processes.

The art also requires apparatus of uncomplex design for hydroenhancing textile materials. Commercial production requires apparatus for continuous fabric hydroenhancing and inline drying of such fabrics under controlled conditions to yield fabrics of uniform specifica- 10

Accordingly, it is a broad object of the invention to provide an improved textile hydroenhancing process and related apparatus for production of a variety of novel woven and knit fabrics having improved characteristics which advance the art.

A more specific object of the invention is to provide a hydroenhancing process for enhancement of fabrics made of spun and spun/filament yarn.

Another object of the invention is to provide a hydroenhancing process having application for the fabrication of novel composite and layered fabrics.

A further object of the invention is to provide a hydroenhancing production line apparatus which is less complex and improved over the prior art.

5  
clude a plurality of cross-directionally ("CD") aligned and spaced manifolds. Columnar jet nozzles having orifice diameters of approximately 0.005 inches with center-to-center spacings of approximately 0.017 inches are mounted approximately 0.5 inches from the screens. At the process energies of the invention, this spacing arrangement provides a curtain of fluid which yields a uniform fabric enhancement. Use of fluid pervious support members which are oriented in offset relation, preferably 45°, effectively limits jet streaks and eliminates reed markings in processed fabrics.

15  
Optimum fabric enhancement results are obtained in fabrics woven or knit of yarns including fibers with deniers and staple lengths in the range of 0.5 to 6.0, and 0.5 to 5 inches, respectively, and yarn counts in the range of 0.5 s to 50 s. Preferred yarn spinning systems of the invention fabrics include cotton spun, wrap spun, wool spun and friction spun.

20  
Other objects, features and advantages of the present invention will be apparent when the detailed description of the preferred embodiments of the invention are considered in conjunction with the drawings which should be construed in an illustrative and not limiting sense as follows:

#### DISCLOSURE OF THE INVENTION

In the present invention, these purposes, as well as others which will be apparent, are achieved generally by providing an apparatus and a related method for hydroenhancing woven and knit fabrics through dynamic fluid action. A hydroenhancing module is employed in the invention in which the fabric is supported on a member and impacted with a fluid curtain under controlled process energies. Enhancement of the fabric is effected by entanglement and intertwining of yarn fibers at cross-over points in the fabric weave or knit. Fabrics enhanced in accordance with the invention have a uniform finish and improved characteristics, such as, edge fray, drape, stability, wrinkle recovery, 30  
40  
45  
abrasion resistance, fabric weight and thickness.

According to the preferred method of the invention, the woven or knit fabric is advanced on a process line through a weft straightener to two in-line fluid modules for first and second stage fabric enhancement. Top and bottom sides of the fabric are respectively supported on members in the modules and impacted by fluid curtains to impart a uniform finish to the fabric. Preferred support members are fluid pervious, include open areas of approximately 25%, and have fine mesh patterns which permit fluid passage without imparting a patterned effect to the fabric. It is a feature of the invention to employ support members in the modules which include fine mesh patterned screens which are arranged in offset relation to one another with respect to the process line. This offset orientation limits fluid streaks and eliminates reed marking in processed fabrics.

55  
First and second stage enhancement is preferably effected by columnar fluid jets which impact the fabric at pressures within the range of 200 to 3000 psi and impart a total energy to the fabric of approximately 0.10 to 2.0 hp-hr/lb.

Following enhancement, the fabric is advanced to a tenter frame which dries the fabric to a specified width under tension to produce a uniform fabric finish.

60  
Advantage in the invention apparatus is obtained by provision of a continuous process line of uncomplex design. The first and second enhancement stations in-

30  
35  
40  
45  
50  
55  
60  
65  
70  
75  
80  
85  
90  
95  
100  
105  
110  
115  
120  
125  
130  
135  
140  
145  
150  
155  
160  
165  
170  
175  
180  
185  
190  
195  
200  
205  
210  
215  
220  
225  
230  
235  
240  
245  
250  
255  
260  
265  
270  
275  
280  
285  
290  
295  
300  
305  
310  
315  
320  
325  
330  
335  
340  
345  
350  
355  
360  
365  
370  
375  
380  
385  
390  
395  
400  
405  
410  
415  
420  
425  
430  
435  
440  
445  
450  
455  
460  
465  
470  
475  
480  
485  
490  
495  
500  
505  
510  
515  
520  
525  
530  
535  
540  
545  
550  
555  
560  
565  
570  
575  
580  
585  
590  
595  
600  
605  
610  
615  
620  
625  
630  
635  
640  
645  
650  
655  
660  
665  
670  
675  
680  
685  
690  
695  
700  
705  
710  
715  
720  
725  
730  
735  
740  
745  
750  
755  
760  
765  
770  
775  
780  
785  
790  
795  
800  
805  
810  
815  
820  
825  
830  
835  
840  
845  
850  
855  
860  
865  
870  
875  
880  
885  
890  
895  
900  
905  
910  
915  
920  
925  
930  
935  
940  
945  
950  
955  
960  
965  
970  
975  
980  
985  
990  
995  
1000  
1005  
1010  
1015  
1020  
1025  
1030  
1035  
1040  
1045  
1050  
1055  
1060  
1065  
1070  
1075  
1080  
1085  
1090  
1095  
1100  
1105  
1110  
1115  
1120  
1125  
1130  
1135  
1140  
1145  
1150  
1155  
1160  
1165  
1170  
1175  
1180  
1185  
1190  
1195  
1200  
1205  
1210  
1215  
1220  
1225  
1230  
1235  
1240  
1245  
1250  
1255  
1260  
1265  
1270  
1275  
1280  
1285  
1290  
1295  
1300  
1305  
1310  
1315  
1320  
1325  
1330  
1335  
1340  
1345  
1350  
1355  
1360  
1365  
1370  
1375  
1380  
1385  
1390  
1395  
1400  
1405  
1410  
1415  
1420  
1425  
1430  
1435  
1440  
1445  
1450  
1455  
1460  
1465  
1470  
1475  
1480  
1485  
1490  
1495  
1500  
1505  
1510  
1515  
1520  
1525  
1530  
1535  
1540  
1545  
1550  
1555  
1560  
1565  
1570  
1575  
1580  
1585  
1590  
1595  
1600  
1605  
1610  
1615  
1620  
1625  
1630  
1635  
1640  
1645  
1650  
1655  
1660  
1665  
1670  
1675  
1680  
1685  
1690  
1695  
1700  
1705  
1710  
1715  
1720  
1725  
1730  
1735  
1740  
1745  
1750  
1755  
1760  
1765  
1770  
1775  
1780  
1785  
1790  
1795  
1800  
1805  
1810  
1815  
1820  
1825  
1830  
1835  
1840  
1845  
1850  
1855  
1860  
1865  
1870  
1875  
1880  
1885  
1890  
1895  
1900  
1905  
1910  
1915  
1920  
1925  
1930  
1935  
1940  
1945  
1950  
1955  
1960  
1965  
1970  
1975  
1980  
1985  
1990  
1995  
2000  
2005  
2010  
2015  
2020  
2025  
2030  
2035  
2040  
2045  
2050  
2055  
2060  
2065  
2070  
2075  
2080  
2085  
2090  
2095  
2100  
2105  
2110  
2115  
2120  
2125  
2130  
2135  
2140  
2145  
2150  
2155  
2160  
2165  
2170  
2175  
2180  
2185  
2190  
2195  
2200  
2205  
2210  
2215  
2220  
2225  
2230  
2235  
2240  
2245  
2250  
2255  
2260  
2265  
2270  
2275  
2280  
2285  
2290  
2295  
2300  
2305  
2310  
2315  
2320  
2325  
2330  
2335  
2340  
2345  
2350  
2355  
2360  
2365  
2370  
2375  
2380  
2385  
2390  
2395  
2400  
2405  
2410  
2415  
2420  
2425  
2430  
2435  
2440  
2445  
2450  
2455  
2460  
2465  
2470  
2475  
2480  
2485  
2490  
2495  
2500  
2505  
2510  
2515  
2520  
2525  
2530  
2535  
2540  
2545  
2550  
2555  
2560  
2565  
2570  
2575  
2580  
2585  
2590  
2595  
2600  
2605  
2610  
2615  
2620  
2625  
2630  
2635  
2640  
2645  
2650  
2655  
2660  
2665  
2670  
2675  
2680  
2685  
2690  
2695  
2700  
2705  
2710  
2715  
2720  
2725  
2730  
2735  
2740  
2745  
2750  
2755  
2760  
2765  
2770  
2775  
2780  
2785  
2790  
2795  
2800  
2805  
2810  
2815  
2820  
2825  
2830  
2835  
2840  
2845  
2850  
2855  
2860  
2865  
2870  
2875  
2880  
2885  
2890  
2895  
2900  
2905  
2910  
2915  
2920  
2925  
2930  
2935  
2940  
2945  
2950  
2955  
2960  
2965  
2970  
2975  
2980  
2985  
2990  
2995  
3000  
3005  
3010  
3015  
3020  
3025  
3030  
3035  
3040  
3045  
3050  
3055  
3060  
3065  
3070  
3075  
3080  
3085  
3090  
3095  
3100  
3105  
3110  
3115  
3120  
3125  
3130  
3135  
3140  
3145  
3150  
3155  
3160  
3165  
3170  
3175  
3180  
3185  
3190  
3195  
3200  
3205  
3210  
3215  
3220  
3225  
3230  
3235  
3240  
3245  
3250  
3255  
3260  
3265  
3270  
3275  
3280  
3285  
3290  
3295  
3300  
3305  
3310  
3315  
3320  
3325  
3330  
3335  
3340  
3345  
3350  
3355  
3360  
3365  
3370  
3375  
3380  
3385  
3390  
3395  
3400  
3405  
3410  
3415  
3420  
3425  
3430  
3435  
3440  
3445  
3450  
3455  
3460  
3465  
3470  
3475  
3480  
3485  
3490  
3495  
3500  
3505  
3510  
3515  
3520  
3525  
3530  
3535  
3540  
3545  
3550  
3555  
3560  
3565  
3570  
3575  
3580  
3585  
3590  
3595  
3600  
3605  
3610  
3615  
3620  
3625  
3630  
3635  
3640  
3645  
3650  
3655  
3660  
3665  
3670  
3675  
3680  
3685  
3690  
3695  
3700  
3705  
3710  
3715  
3720  
3725  
3730  
3735  
3740  
3745  
3750  
3755  
3760  
3765  
3770  
3775  
3780  
3785  
3790  
3795  
3800  
3805  
3810  
3815  
3820  
3825  
3830  
3835  
3840  
3845  
3850  
3855  
3860  
3865  
3870  
3875  
3880  
3885  
3890  
3895  
3900  
3905  
3910  
3915  
3920  
3925  
3930  
3935  
3940  
3945  
3950  
3955  
3960  
3965  
3970  
3975  
3980  
3985  
3990  
3995  
4000  
4005  
4010  
4015  
4020  
4025  
4030  
4035  
4040  
4045  
4050  
4055  
4060  
4065  
4070  
4075  
4080  
4085  
4090  
4095  
4100  
4105  
4110  
4115  
4120  
4125  
4130  
4135  
4140  
4145  
4150  
4155  
4160  
4165  
4170  
4175  
4180  
4185  
4190  
4195  
4200  
4205  
4210  
4215  
4220  
4225  
4230  
4235  
4240  
4245  
4250  
4255  
4260  
4265  
4270  
4275  
4280  
4285  
4290  
4295  
4300  
4305  
4310  
4315  
4320  
4325  
4330  
4335  
4340  
4345  
4350  
4355  
4360  
4365  
4370  
4375  
4380  
4385  
4390  
4395  
4400  
4405  
4410  
4415  
4420  
4425  
4430  
4435  
4440  
4445  
4450  
4455  
4460  
4465  
4470  
4475  
4480  
4485  
4490  
4495  
4500  
4505  
4510  
4515  
4520  
4525  
4530  
4535  
4540  
4545  
4550  
4555  
4560  
4565  
4570  
4575  
4580  
4585  
4590  
4595  
4600  
4605  
4610  
4615  
4620  
4625  
4630  
4635  
4640  
4645  
4650  
4655  
4660  
4665  
4670  
4675  
4680  
4685  
4690  
4695  
4700  
4705  
4710  
4715  
4720  
4725  
4730  
4735  
4740  
4745  
4750  
4755  
4760  
4765  
4770  
4775  
4780  
4785  
4790  
4795  
4800  
4805  
4810  
4815  
4820  
4825  
4830  
4835  
4840  
4845  
4850  
4855  
4860  
4865  
4870  
4875  
4880  
4885  
4890  
4895  
4900  
4905  
4910  
4915  
4920  
4925  
4930  
4935  
4940  
4945  
4950  
4955  
4960  
4965  
4970  
4975  
4980  
4985  
4990  
4995  
5000  
5005  
5010  
5015  
5020  
5025  
5030  
5035  
5040  
5045  
5050  
5055  
5060  
5065  
5070  
5075  
5080  
5085  
5090  
5095  
5100  
5105  
5110  
5115  
5120  
5125  
5130  
5135  
5140  
5145  
5150  
5155  
5160  
5165  
5170  
5175  
5180  
5185  
5190  
5195  
5200  
5205  
5210  
5215  
5220  
5225  
5230  
5235  
5240  
5245  
5250  
5255  
5260  
5265  
5270  
5275  
5280  
5285  
5290  
5295  
5300  
5305  
5310  
5315  
5320  
5325  
5330  
5335  
5340  
5345  
5350  
5355  
5360  
5365  
5370  
5375  
5380  
5385  
5390  
5395  
5400  
5405  
5410  
5415  
5420  
5425  
5430  
5435  
5440  
5445  
5450  
5455  
5460  
5465  
5470  
5475  
5480  
5485  
5490  
5495  
5500  
5505  
5510  
5515  
5520  
5525  
5530  
5535  
5540  
5545  
5550  
5555  
5560  
5565  
5570  
5575  
5580  
5585  
5590  
5595  
5600  
5605  
5610  
5615  
5620  
5625  
5630  
5635  
5640  
5645  
5650  
5655  
5660  
5665  
5670  
5675  
5680  
5685  
5690  
5695  
5700  
5705  
5710  
5715  
5720  
5725  
5730  
5735  
5740  
5745  
5750  
5755  
5760  
5765  
5770  
5775  
5780  
5785  
5790  
5795  
5800  
5805  
5810  
5815  
5820  
5825  
5830  
5835  
5840  
5845  
5850  
5855  
5860  
5865  
5870  
5875  
5880  
5885  
5890  
5895  
5900  
5905  
5910  
5915  
5920  
5925  
5930  
5935  
5940  
5945  
5950  
5955  
5960  
5965  
5970  
5975  
5980  
5985  
5990  
5995  
6000  
6005  
6010  
6015  
6020  
6025  
6030  
6035  
6040  
6045  
6050  
6055  
6060  
6065  
6070  
6075  
6080  
6085  
6090  
6095  
6100  
6105  
6110  
6115  
6120  
6125  
6130  
6135  
6140  
6145  
6150  
6155  
6160  
6165  
6170  
6175  
6180  
6185  
6190  
6195  
6200  
6205  
6210  
6215  
6220  
6225  
6230  
6235  
6240  
6245  
6250  
6255  
6260  
6265  
6270  
6275  
6280  
6285  
6290  
6295  
6300  
6305  
6310  
6315  
6320  
6325  
6330  
6335  
6340  
6345  
6350  
6355  
6360  
6365  
6370  
6375  
6380  
6385  
6390  
6395  
6400  
6405  
6410  
6415  
6420  
6425  
6430  
6435  
6440  
6445  
6450  
6455  
6460  
6465  
6470  
6475  
6480  
6485  
6490  
6495  
6500  
6505  
6510  
6515  
6520  
6525  
6530  
6535  
6540  
6545  
6550  
6555  
6560  
6565  
6570  
6575  
6580  
6585  
6590  
6595  
6600  
6605  
6610  
6615  
6620  
6625  
6630  
6635  
6640  
6645  
6650  
6655  
6660  
6665  
6670  
6675  
6680  
6685  
6690  
6695  
6700  
6705  
6710  
6715  
6720  
6725  
6730  
6735  
6740  
6745  
6750  
6755  
6760  
6765  
6770  
6775  
6780  
6785  
6790  
6795  
6800  
6805  
6810  
6815  
6820  
6825  
6830  
6835  
6840  
6845  
6850  
6855  
6860  
6865  
6870  
6875  
6880  
6885  
6890  
6895  
6900  
6905  
6910  
6915  
6920  
6925  
6930  
6935  
6940  
6945  
6950  
6955  
6960  
6965  
6970  
6975  
6980  
6985  
6990  
6995  
7000  
7005  
7010  
7015  
7020  
7025  
7030  
7035  
7040  
7045  
7050  
7055  
7060  
7065  
7070  
7075  
7080  
7085  
7090  
7095  
7100  
7105  
7110  
7115  
7120  
7125  
7130  
7135  
7140  
7145  
7150  
7155  
7160  
7165  
7170  
7175  
7180  
7185  
7190  
7195  
7200  
7205  
7210  
7215  
7220  
7225  
7230  
7235  
7240  
7245  
7250  
7255  
7260  
7265  
7270  
7275  
7280  
7285  
7290  
7295  
7300  
7305  
7310  
7315  
7320  
7325  
7330  
7335  
7340  
7345  
7350  
7355  
7360  
7365  
7370  
7375  
7380  
7385  
7390  
7395  
7400  
7405  
7410  
7415  
7420  
7425  
7430  
7435  
7440  
7445  
7450  
7455  
7460  
7465  
7470  
7475  
7480  
7485  
7490  
7495  
7500  
7505  
7510  
7515  
7520  
7525  
7530  
7535  
7540  
7545  
7550  
7555  
7560  
7565  
7570  
7575  
7580  
7585  
7590  
7595  
7600  
7605  
7610  
7615  
7620  
7625  
7630  
7635  
7640  
7645  
7650  
7655  
7660  
7665  
7670  
7675  
7680  
7685  
7690  
7695  
7700  
7705  
7710  
7715  
7720  
7725  
7730  
7735  
7740  
7745  
7750  
7755  
7760  
7765  
7770  
7775  
7780  
7785  
7790  
7795  
7800  
7805  
7810  
7815  
7820  
7825  
7830  
7835  
7840  
7845  
7850  
7855  
7860  
7865  
7870  
7875  
7880  
7885  
7890  
7895  
7900  
7905  
7910  
7915  
7920  
7925  
7930  
7935  
7940  
7945  
7950  
7955  
7960  
7965  
7970  
7975  
7980  
7985  
7990  
7995  
8000  
8005  
8010  
8015  
8020  
8025  
8030  
8035  
8040  
8045  
8050  
8055  
8060  
8065  
8070  
8075  
8080  
8085  
8090  
8095  
8100  
8105  
8110  
8115  
8120  
8125  
8130  
8135  
8140  
8145  
8150  
8155  
8160  
8165  
8170  
8175  
8180  
8185  
8190  
8195  
8200  
8205  
8210  
8215  
8220  
8225  
8230  
8235  
8240  
8245  
8250  
8255  
8260  
8265  
8270  
8275  
8280  
8285  
8290  
8295  
8300  
8305  
8310  
8315  
8320  
8325  
8330  
8335  
8340  
8345  
8350  
8355  
8360  
8365  
8370  
8375  
8380  
8385  
8390  
8395  
8400  
8405  
8410<br

fabric of FIGS. 12A and B hydroenhanced in accordance with the invention;

FIG. 14 is a photomacrograph at 0.09X magnification of a control and hydroenhanced acrylic fabric strips, the fabric of FIGS. 7A and B, showing the reduction in fabric torque achieved in the invention process;

FIGS. 15 A-C are photomacrographs at 0.23X magnification, respectively, of the woven acrylic fabrics of FIGS. 5, 7 and 8, 0 comprised of wrap spun and open end wool spun yarns, showing washability and wrinkle characteristics of control and processed fabrics;

FIGS. 16A and B are photomacrographs at approximately 1X magnification of control and hydroenhanced acrylic fabric including wrap spun polyester yarns, showing washability and surface durability characteristics results obtained in the invention process;

FIGS. 17A and B are photomacrographs at approximately 1X magnification of control and hydroenhanced 100% polyester fabric which includes slub yarns, showing washability surface durability characteristics results obtained in the invention process

FIGS. 18A and B are photomacrographs at IX magnification of control and hydroenhanced 80% wool and 20% nylon fabric, showing washability surface durability characteristics results obtained in the invention process;

FIG. 19 is a schematic view of an alternative production line apparatus for the hydroenhancement of woven and knit fabrics in accordance with the invention;

FIG. 20 illustrates a composite fabric including napped fabric components which are bonded into an integral structure employing the hydroenhancing process of the invention; and

FIG. 21A and B, respectively, are enlarged schematic illustrations, of a nonwoven-textile fabric composite before and subsequent to enhancement and lamination in accordance with the invention process.

#### BEST MODE OF CARRYING OUT THE INVENTION

With further reference to the drawings, FIG. 1 illustrates a preferred embodiment of a production line of the invention, generally designated 10, for hydroenhancement of a fabric 12 including spun and/or spun-filament yarns. The line includes a conventional weft straightener 14, flat and drum enhancing modules 16, 18, and a tenter frame 20.

Modules 16, 18 effect two sided enhancement of the fabric through fluid entanglement and bulking of fabric yarns. Such entanglement is imparted to the fabric in areas of yarn crossover or intersection. Control of process energies and provision of a uniform curtain of fluid produces fabrics having a uniform finish and improved characteristics including, edge fray, torque, wrinkle recovery, cupping, drape, stability, abrasion resistance, fabric weight and thickness.

#### METHOD AND MECHANISM OF THE ENHANCING MODULES

Fabric is advanced through the weft straightener 14 which aligns the fabric weft prior to processing in enhancement modules 16, 18. Following hydroenhancement, the fabric is advanced to the tenter frame 20, which is of conventional design, where it is dried under tension to produce a uniform fabric of specified width.

Module 16 includes a first support member 22 which is supported on an endless conveyor means including rollers 24 and drive means (not shown) for rotation of

the rollers. Preferred line speeds for the conveyor are in the range of 10 to 500 ft/min. Line speeds are adjusted in accordance with process energy requirements which vary as a function of fabric type and weight.

Support member 22, which preferably has a flat configuration, includes closely spaced fluid pervious open areas 26. A preferred support member 22, shown in FIG. 2A, is a 36×29 90° mesh plain weave having a 23.7% open area, fabricated of polyester warp and shute round wire. Support member 22 is a tight seamless weave which is not subject to angular displacement or snag. Specifications for the screen, which is manufactured by Albany International, Appleton Wire Division, P.O. Box 1939, Appleton, Wis. 54913 are set forth in Table I.

TABLE I

| Property   | Support Screen Specifications |                       |
|------------|-------------------------------|-----------------------|
|            | 36 × 29 90° flat mesh         | 40 × 40 45° drum mesh |
| Wire       | polyester                     | stainless steel       |
| Warp wire  | .0157                         | 0.010                 |
| Shute wire | .0157                         | 0.010                 |
| Weave type | plain                         | plain                 |
| Open area  | 23.7%                         | 36%                   |

Module 16 also includes an arrangement of parallel and spaced manifolds 30 oriented in a cross-direction ("CD") relative to movement of the fabric 12. The manifolds which are spaced approximately 8 inches apart each include a plurality of closely aligned and spaced columnar jet orifices 32 which are spaced approximately 0.5 inches from the support member 22.

The jet orifices have diameters and center-to-center spacings in the range of 0.005 to 0.010 inches and 0.017 to 0.034 inches, respectively, and are designed to impact the fabric with fluid pressures in the range of 200 to 3000 psi. Preferred orifices have diameters of approximately 0.005 inches with center-to-center spacings of approximately 0.017 inches.

This arrangement of fluid jets provides a curtain of fluid entangling streams which yield optimum enhancement in the fabric. Energy input to the fabric is cumulative along the line and preferably set at approximately the same level in modules 16, 18 (two stage system) to impart uniform enhancement to top and bottom surfaces of the fabric. Effective first stage enhancement of fabric yarn is achieved at an energy output of at least 0.05 hp-hr/lb and preferably in the range of 0.1 to 2.0 hp-hr/lb.

Following the first stage enhancement, the fabric is advanced to module 18 which enhances the other side of the fabric. Module 18 includes a second support member 34 of cylindrical configuration which is supported on a drum. The member 34 includes closely spaced fluid pervious open areas 36 which comprise approximately 36% of the screen area. A preferred support member 34, shown in FIG. 2B, is a 40×40 45° mesh stainless steel screen, manufactured by Appleton Wire, having the specifications set forth in Table I.

Module 18 functions in the same manner as the planar module 16. Manifolds 30 and jet orifices 32 are provided which have substantially the same specifications as in the first stage enhancement module. Fluid energy to the fabric of at least 0.5 hp-hr/lb and preferably in the range of 0.1 to 2.0 hp-hr/lb effects second stage enhancement.

Conventional weaving processes impart reed marks to fabrics. Illustrations of such markings are shown in FIGS. 3A and 4A which are photomicrographs at 10X

and 16X magnification of a polyester LIBBEY brand fabric style no. S/x-A805 (see Table II). Reed marks in FIGS. 3A and 4A are designated by the letter "R".

The invention overcomes this defect in conventional weaving processes through use of a single and preferably two stage hydroenhancement process. Advantage is obtained in the invention process by orienting the drum support member 34 in offset relation, preferably 45°, relative to machine direction ("MD") of the hydroenhancing line. See FIGS. 2A and B.

Support members 22 and 34 are preferably provided with fine mesh open areas which are dimensioned to effect fluid passage through the members without imparting a patterned effect to the fabric. The preferred members have an effective open area for fluid passage in the range of 17-40%.

Comparison of the control and processed polyester fabric of FIGS. 3A, B and 4A, B illustrates the advantages obtained through use of the enhancement process. Reed marks R in control polyester fabric are essentially eliminated through enhancement of the fabric. The offset screen arrangement is also effective in diminishing linear jet streak markings associated with the enhancement process.

#### EXAMPLES I-XIII

FIGS. 3-15 illustrate representative woven and knit fabrics enhanced in accordance with the method of the invention, employing test conditions which simulate the line of FIG. 1 (hereinafter the "Prototype FIG. 1 line"). Table II sets forth specifications for the fabrics illustrated in the drawings.

As in the FIG. 1 line, the test manifolds 30 were spaced approximately 8 inches apart in modules 16, 18, and provided with densely packed columnar jet orifices 32 of approximately 60/inch. Orifices 32 each had a diameter of 0.005 inches and were spaced approximately 0.5 inches from the first and second support members 22, 34.

The process line of FIG. 1 includes enhancement modules 16, 18 which, respectively, are provided with six manifolds. In the Examples, modules 16, 18 were each fitted with two manifolds 34. To simulate line conditions, the fabrics were advanced through multiple runs on the line. Three processing runs in each two manifold module was deemed to be equivalent to a six manifold module.

Fabrics were hydroenhanced at process pressures of approximately 1500 psi. Line speed and cumulative energy output to the modules were respectively maintained at approximately 30 fpm and 0.46 hp-hr/lb. Adjustments in the line speed and fluid pressure were made to accommodate differences in fabric weight for uniform processing and to maintain the preferred energy level.

Fabrics processed in the Examples exhibited marked enhancement in aesthetic appearance and quality including, characteristics such as cover, bloom, abrasion resistance, drape, stability, and reduction in seam slip page, and edge fray.

Tables III-XI set forth data for fabrics enhanced in accordance with invention on the test process line. Standard testing procedures of The American Society for Testing and Materials (ASTM) were employed to test control and processed characteristics of fabrics. Data set forth in the Tables was generated in accordance with the following ASTM standards:

| Fabric Characteristic | ASTM Standard                       |
|-----------------------|-------------------------------------|
| Weight                | D3776-79                            |
| Thickness             | D1777-64 (Ames Tester)              |
| Tensile Load          | D1682-64 (1975)<br>(Cut strip/grab) |
| Elongation            | D1682-64 (1975)                     |
| Air Permeability      | D737-75 (1980) (Frazier)            |
| Thread Count          | D3775-79                            |
| Ball Burst            | D3787-80A                           |
| Slippage              | D4159-82                            |
| Tongue Tear           | D2261-71                            |
| Wrinkle Recovery      | D1295-67 (1972)                     |
| Abrasion Resistance   | D3884-80                            |
| Pilling               | D3514-81                            |

Washability tests were conducted in accordance with the following procedure. Weight measurements ("before wash") were taken of control and processed fabric samples each having a dimension of 8.5"×11" (8.5" fill direction and 11" warp direction). The samples were then washed and dried in conventional washer and dryers three consecutive times and "after wash" measurements were taken. The percent weight loss of the pre and post wash samples was determined in accordance the following formula:

$$\% \text{ weight loss} = D/B \times 100$$

where, B=before wash sample weight; A=after wash sample weight; and D=B-A.

Photomicrographs of the fabrics, FIGS. 4-15, illustrate the enhancement in fabric cover obtained in the invention. Attention is directed to open areas in the unprocessed fabrics, photographs designated A, these areas are of reduced size in the processed fabrics in the photographs designated B. Hydroenhancement caused fabric yarns to bloom and entangle at cross-over points, filling in open areas to improve cover and reduce air permeability in the fabrics.

FIGS. 12 and 13 are photomicrographs of a HYTEX brand wall covering fabric, manufactured by Hytex, Inc, Randolph, Mass. A multi-textured surface appearance of the fabric is provided by yarns which are woven through discrete areas of the front fabric surface. Free floating weave stitches, designated by the letter "S" in FIGS. 12B and 13B, are formed on the backside of the fabric.

Hydroenhancement of HYTEX wall covering fabric secured the free-floating stitches S to the fabric backside enhancing fabric stability and cover. See FIGS. 12B, 13B. In wall covering applications, fabric enhancement and associated stabilizing effects reduces or eliminates the need for adhesive backcoatings. Enhancement of the fabric also limits wicking of wall cover application adhesives through the fabric. Further advantage is obtained when enhanced fabrics are used in acoustic applications; elimination of backcoating reduces sound reflection and furthers efficient transmission of sound through the fabric.

TABLE II

| Fabric Specifications              |  |            |
|------------------------------------|--|------------|
| Fiber Brand and Style Designation  |  | FIG(S)     |
| NOMEX S/x-A805*                    |  | 3A,B, 4A,B |
| Fiber: 2 denier-1.9 inch           |  |            |
| Yarn: Open end cotton spun 17s     |  |            |
| LIBBEY S/022**                     |  | 5A,B       |
| Warp:                              |  |            |
| Fiber: 3 denier - 1.5 inch acrylic |  |            |

TABLE II-continued

| Fabric Specifications                                                             |        | FIG(S.)                                                                                                                                       |
|-----------------------------------------------------------------------------------|--------|-----------------------------------------------------------------------------------------------------------------------------------------------|
| Fiber Brand and Style Designation                                                 |        |                                                                                                                                               |
| Yarn: Open end cotton spun 9s<br>28 ends per inch                                 |        | 5                                                                                                                                             |
| Fill:<br>Fiber: 3 denier - 3 inch acrylic                                         |        | 27                                                                                                                                            |
| Yarn: Open end wool spun 4s<br>14, 16 or 18 picks per inch                        |        | 28                                                                                                                                            |
| LIBBEY S/x-1160                                                                   | 6A,B   | +3.7                                                                                                                                          |
| Fiber: 3 denier-3 inch acrylic                                                    |        | Seam Slippage (lbs/in)                                                                                                                        |
| Yarn: Wrap spun w/100 den<br>textured polyester 4s                                |        | warp                                                                                                                                          |
| 14 ends $\times$ 16 picks per inch                                                |        | 5                                                                                                                                             |
| LIBBEY S/406                                                                      | 7A,B   | fill                                                                                                                                          |
| 14A,B                                                                             |        | 7                                                                                                                                             |
| Warp:<br>Fiber: 3 denier - 1.5 inch acrylic                                       |        | Tongue Tear (lbs)                                                                                                                             |
| Yarn: Open end cotton spun 9s<br>28 ends per inch                                 |        | warp                                                                                                                                          |
| Fill:<br>Fiber: 3 denier - 3 inch acrylic                                         |        | 18                                                                                                                                            |
| Yarn: Hollow spun 6 twists/inch 4s<br>14, 16 or 18 picks per inch                 |        | fill                                                                                                                                          |
| LIBBEY S/152                                                                      | 8A,B   | 21                                                                                                                                            |
| Warp:<br>Fiber: 3 denier - 2.5 inch acrylic                                       |        | Wt. Loss In Wash (%)                                                                                                                          |
| Yarn: Open end cotton spun 4s<br>14 ends per inch                                 |        | 37                                                                                                                                            |
| Fill:<br>Fiber: 3 denier - 3 inch acrylic                                         |        | 123°                                                                                                                                          |
| Yarn: Open end wool spun 2.6s<br>14, 16 or 18 picks per inch                      |        | 138°                                                                                                                                          |
| Guilford Wool/Nylon<br>80% wool/20% nylon                                         | 9A,B   | (recovery angle)                                                                                                                              |
| Polyester/cotton (53/47)<br>Weight: 10 ounces/yd <sup>2</sup>                     | 10A,B  | *Under ASTM test standards (D1295-67) improvements in the wrinkle recovery of<br>a fabric are indicated by an increase in the recovery angle. |
| Yarn: Spun Filament<br>Weave: 3 $\times$ 1 Twill<br>Thread Count: 120 $\times$ 38 |        |                                                                                                                                               |
| 50% Polyester/50% cotton Doubleknit                                               | 11A,B  |                                                                                                                                               |
| Yarn: wrap spun with 100<br>denier polyester wrap                                 |        |                                                                                                                                               |
| HYTEX Wall covering***                                                            | 12, 13 |                                                                                                                                               |

\*LIBBEY is a trademark of W. S. Libbey Co., One Mill Street, Lewiston, ME 04240.

\*\*NOMEX is a trademark of E.I. Du Pont de Nemours and Company, Wilmington, Del.

\*\*\*HYTEX is a trademark of Hytex, Inc., Randolph, MA.

TABLE III

| Nomex A805 - FIG. 4                               |           |          |
|---------------------------------------------------|-----------|----------|
| Control                                           | Processed | % Change |
| Weight (gsy)                                      | 195       | 197      |
| Thickness (mils)                                  | 42        | 42       |
| Air Perm. (ft <sup>3</sup> /ft <sup>2</sup> /min) | 331       | 156      |
| Strip Tensile (lbs/in)                            |           | -52.9    |
| warp                                              | 115       | 132      |
| fill                                              | 59        | 47       |
| Elongation (%)                                    |           | +14.8    |
| warp                                              | 48        | 50       |
| fill                                              | 62        | 71       |

TABLE IV

| 022/6075 (16 ppi) - FIG. 5                        |           |          |
|---------------------------------------------------|-----------|----------|
| Control                                           | Processed | % Change |
| Weight (gsy)                                      | 158       | 165      |
| Thickness (mils)                                  | 48        | 49       |
| Air Perm. (ft <sup>3</sup> /ft <sup>2</sup> /min) | 406       | 259      |
| Strip Tensile (lbs/in)                            |           | -36.2    |
| warp                                              | 34        | 36       |
| fill                                              | 37        | 31       |
| Elongation (%)                                    |           | +5.9     |
| warp                                              | 33        | 27       |

TABLE IV-continued

| 022/6075 (16 ppi) - FIG. 5 |         |           |          |
|----------------------------|---------|-----------|----------|
|                            | Control | Processed | % Change |
| 5                          | 27      | 28        | +3.7     |
| Seam Slippage (lbs/in)     |         |           |          |
| warp                       | 5       | 60        | +1100.0  |
| fill                       | 7       | 55        | +685.7   |
| Tongue Tear (lbs)          |         |           |          |
| warp                       | 18      | 10        | -44.4    |
| fill                       | 21      | 8         | -61.9    |
| Wt. Loss In Wash (%)       | 37      | 5         | -86.5    |
| Wrinkle Recovery*          | 123°    | 138°      | +12.2    |
| (recovery angle)           |         |           |          |

\*Under ASTM test standards (D1295-67) improvements in the wrinkle recovery of  
a fabric are indicated by an increase in the recovery angle.

TABLE V

| Libbey S/x-1160 - FIG. 6                          |              |           |          |
|---------------------------------------------------|--------------|-----------|----------|
|                                                   | Control      | Processed | % Change |
| 20                                                | Weight (gsy) | 146.8     | 160.2    |
| Thickness (mils)                                  | 38.1         | 52.7      | 38.3     |
| Air Perm. (ft <sup>3</sup> /ft <sup>2</sup> /min) | 457.2        | 188.5     | -58.8    |
| Grab Tensile (lbs/in)                             |              |           |          |
| warp                                              | 80.2         | 89.3      | 11.4     |
| fill                                              | 105.0        | 111.4     | 6.1      |
| Elongation (%)                                    |              |           |          |
| warp                                              | 30.0         | 34.0      | 13.3     |
| fill                                              | 32.0         | 46.0      | 43.8     |
| Ball Burst (lbs)                                  | 190          | 157       | -17.4    |

TABLE VI

| 406/6075 (16 ppi) - FIG. 7                        |              |           |          |
|---------------------------------------------------|--------------|-----------|----------|
|                                                   | Control      | Processed | % Change |
| 35                                                | Weight (gsy) | 159       | 166      |
| Thickness (mils)                                  | 48           | 50        | +4.2     |
| Air Perm. (ft <sup>3</sup> /ft <sup>2</sup> /min) | 351          | 184       | -47.6    |
| Strip Tensile (lbs/in)                            |              |           |          |
| warp                                              | 42           | 36        | -14.3    |
| fill                                              | 66           | 58        | -12.1    |
| Elongation (%)                                    |              |           |          |
| warp                                              | 23           | 31        | +34.8    |
| fill                                              | 49           | 33        | -32.7    |
| Seam Slippage (lbs)                               |              |           |          |
| warp                                              | 29           | 36        | +89.5    |
| fill                                              | 21           | 76        | +261.9   |
| Tongue Tear (lbs)                                 |              |           |          |
| warp                                              | 23           | 18        | -21.7    |
| fill                                              | 19           | 15        | -1.1     |
| Wt. Loss In Wash (%)                              | 28           | 4         | -85.7    |
| Wrinkle Recovery                                  | 140°         | 148°      | +5.7     |
| (recovery angle)                                  |              |           |          |

TABLE VII

| 152/6076 (16 ppi) - FIG. 8                        |              |           |          |
|---------------------------------------------------|--------------|-----------|----------|
|                                                   | Control      | Processed | % Change |
| 55                                                | Weight (gsy) | 231       | 257      |
| Thickness (mils)                                  | 259          | 238       | -8.1     |
| Air Perm. (ft <sup>3</sup> /ft <sup>2</sup> /min) | 204          | 106       | -48.0    |
| Strip Tensile (lbs/in)                            |              |           |          |
| warp                                              | 48           | 58        | +20.8    |
| fill                                              | 56           | 72        | +28.6    |
| Elongation (%)                                    |              |           |          |
| warp                                              | 33           | 33        | 0        |
| fill                                              | 34           | 39        | +14.7    |
| Seam Slippage (lbs)                               |              |           |          |
| warp                                              | 64           | 81        | +26.6    |
| fill                                              | 78           | 112       | +43.6    |
| Tongue Tear (lbs)                                 |              |           |          |

TABLE VII-continued

| 152/6076 (16 ppi) - FIG. 8        |         |           |          |
|-----------------------------------|---------|-----------|----------|
|                                   | Control | Processed | % Change |
| warp                              | 21      | 18        | -14.3    |
| fill                              | 17      | 15        | -11.8    |
| Wt. Loss In Wash (%)              | —       | —         | —        |
| Wrinkle Recovery (recovery angle) | 117°    | 136°      | +16.2    |

TABLE VIII

| Guilford Wool (80% wool/20% nylon) - FIG. 9 |         |         |          |
|---------------------------------------------|---------|---------|----------|
|                                             | Control | Process | % Change |
| Air Perm.                                   | 243     | 147     | -39.5    |

reduction test of FIGS. 14A, B employed fabric strips 84" long and 3.5" wide, which were suspended vertically without restraint. Torque was measured with reference to the angle of fabric twist from a flat support surface. As can be seen in the photographs, a torque of 90° in the unprocessed fabric, FIG. 14A, was eliminated in the enhancement process.

FIGS. 15A-C are macrophotographs of control and processed acrylic fabrics, LIBBEY style nos. 022, 406 and 152, respectively, which were tested for washability. Unprocessed fabrics exhibited excessive fraying and destruction, in contrast to the enhanced fabrics which exhibit limited fraying and yarn (weight) loss. Table XI sets forth washability test weight loss data.

15

TABLE XI

TABLE IXA

| Spun/Filament - Bottom Weights - FIG. 10            |           |          |           |          |           |          |           |          |
|-----------------------------------------------------|-----------|----------|-----------|----------|-----------|----------|-----------|----------|
|                                                     | Sample #1 |          | Sample #2 |          | Sample #3 |          | Sample #4 |          |
|                                                     | Control   | Proc     | Control   | Proc     | Control   | Proc     | Control   | Proc     |
| Weight (g/sy)                                       | 259.2     | 275.4    | 240.3     | 248.4    | 286.2     | 297.2    | 267.3     | 280.8    |
| Thickness (mils)                                    | 39.7      | 39.2     | 35.0      | 35.3     | 44.2      | 41.5     | 40.0      | 38.0     |
| Strip Tensiles (lbs./in.)                           |           |          |           |          |           |          |           |          |
| Warp                                                | 206.98    | 208.87   | 195.50    | 200.86   | 183.09    | 189.95   | 206.43    | 207.87   |
| Fill                                                | 85.55     | 56.23    | 84.21     | 71.83    | 80.88     | 83.01    | 80.16     | 82.14    |
| Normalized Tensiles (lbs./in.)                      |           |          |           |          |           |          |           |          |
| Warp                                                | 7.98      | 7.58     | 8.05      | 8.09     | 6.40      | 6.39     | 7.65      | 7.40     |
| Fill                                                | 3.30      | 2.04     | 2.54      | 2.89     | 2.83      | 2.79     | 3.03      | 2.93     |
| Elongation (%)                                      |           |          |           |          |           |          |           |          |
| Warp                                                | 42.0      | 55.3     | 36.5      | 39.1     | 40.9      | 43.5     | 46.1      | 51.2     |
| Fill                                                | 23.6      | 25.6     | 24.0      | 20.0     | 23.5      | 20.3     | 22.9      | 22.4     |
| Air Perm. (ft. <sup>3</sup> /ft. <sup>2</sup> /min) | 50.9      | 27.3     | 43.5      | 28.8     | 45.8      | 21.8     | 51.4      | 25.4     |
| Thread Count (wxf)                                  | 120 × 40  | 120 × 41 | 120 × 45  | 120 × 45 | 120 × 38  | 120 × 42 | 120 × 42  | 120 × 43 |
| Mullen Burst (lbs.)                                 | 161.2     | 222.2    | 187.2     | 228.8    | 161.0     | 217.8    | 205.0     | 242.2    |
| Normalized Burst (lbs./g × 10 <sup>2</sup> )        | 62.2      | 80.7     | 77.9      | 92.1     | 56.2      | 73.3     | 76.7      | 86.3     |

TABLE IXB

| Abrasion - Spun Filament-Bottom Weights - FIG. 10                    |                   |                  |                 |        |               |
|----------------------------------------------------------------------|-------------------|------------------|-----------------|--------|---------------|
| ASTM Standard - Twill side up; 500 cycles; 500 g weight; H-18 wheels |                   |                  |                 |        |               |
| Sample                                                               | Weight Before (g) | Weight After (g) | Weight Loss (g) | % Loss | % Improvement |
| 1C                                                                   | 3.32              | 3.02             | 0.30            | 9.0    |               |
| 1P                                                                   | 3.36              | 3.13             | 0.23            | 6.9    | 23%           |
| 2C                                                                   | 4.64              | 4.16             | 0.48            | 10.4   |               |
| 2P                                                                   | 4.83              | 4.57             | 0.26            | 5.4    | 48%           |
| 3C                                                                   | 4.73              | 4.47             | 0.26            | 5.5    |               |
| 3P                                                                   | 4.91              | 5.13             | 0.22            | 4.5    | 18%           |
| 4C                                                                   | 4.47              | 4.18             | 0.29            | 6.5    |               |
| 4P                                                                   | 4.71              | 4.53             | 0.18            | 3.8    | 41%           |

40

022, 406, 152 - FIGS. 15A-C  
Percent Weight Loss  
(3 wash/dry cycles)

| Sample | Control | Processed |
|--------|---------|-----------|
| 022    | 36.5    | 5.0       |
| 406    | 28.0    | 4.0       |
| 152    | 28.1    | 7.2       |

In the foregoing Examples, the enhancement process of the invention is shown to yield improved textile finishing features such as, surface cover, abrasion resistance, wrinkle recovery, tensile strength and air permeability. Additional fabric features which may be obtained in the invention include, enhancement of fabric surface durability, absorption and adsorption, and shrinkage reduction. Further, advantageous fabric features are obtained in particular material applications of the invention enhancement process. For example, it has been found that enhancement of wool fabrics yields dense and compact fabrics which are shrink resistant. In another application of the invention technology improvements in fabric flame retardancy have been obtained in the processing of polyester based fabrics.

Examples illustrating further applications and embodiments of the invention are set forth below. As in the prior Examples, fabrics were processed on the Prototype FIG. 1 line described in the previous Examples. Fabrics were hydroenhanced at process pressures of approximately 1500 psi. Line speed and cumulative

| Doubleknit - FIG. 11                               |         |           |          |
|----------------------------------------------------|---------|-----------|----------|
|                                                    | Control | Processed | % Change |
| Air Perm. (ft. <sup>3</sup> /ft. <sup>2</sup> min) | 113.1   | 95.1      | -15.9    |
| Abrasion ASTM (D-3884-80): 250 Cycles, H-18 wheel  | 1.0     | 0.6       | -40.0    |
| Pilling (1-5 rating)                               | 4.3     | 4.3       | 0        |
| ASTM (D-3914-81): 300 cycles                       |         |           |          |

FIGS. 14A, B are photomacrophotographs of control and processed acrylic vertical blind fabric, manufactured by W. S. Libbey, style designation S/406. Enhancement of the fabric reduces fabric torque which is particularly advantageous in vertical blind applications. The torque

65

energy output to the entanglement modules were respectively maintained at approximately 30 fpm and 0.5 hp-hr/lb. Adjustments in the line speed and fluid pressure were made to accommodate differences in fabric weight for uniform processing and to maintain the preferred energy levels.

**EXAMPLE XIV**  
**Fabric Surface Durability**

Conventional finishing processes for imparting surface durability to fabrics employ chemical binders which lock fabric fibers into stable orientations. Such "durable" or "permanent" press processes stiffen fabric finishes and adversely effect the hand and drape characteristics in fabrics. The hydroenhancement process of

shrinkage measurements were recorded with reference to line markings. As in prior Example XIV, laundering conditions approximated standards set forth in the AATCC Technical Manual, Test Method 124-1984.

5 Comparison of processed and control test data demonstrates that the invention enhancement obtains a measurable reduction in shrink resistance. For example, after five wash/dry cycles, enhanced 65% wool/PET% exhibits a 6.9 percent shrinkage as compared to

10 14.4 percent shrinkage in an unprocessed control.

Attention is directed Table XIV which sets forth data for shrinkage in wool fabrics. It will be seen that stabilization in wool fabrics provides a "washable wool" without requirement of conventional chemical finishing treatment.

TABLE XII

| Original Sample<br>10" x 10" | SHRINKAGE - 5 WASH/DRY CYCLES<br>Warp/Fill (W/F) Measurements |       |                      |       |                           |       |
|------------------------------|---------------------------------------------------------------|-------|----------------------|-------|---------------------------|-------|
|                              | Measurement<br>After Wash<br>(inches)                         |       | Percent<br>Shrinkage |       | Percent Area<br>Shrinkage |       |
|                              | Sample                                                        | Cont. | Proc.                | Cont. | Proc.                     | Cont. |
| Greige Cotton                | W                                                             | 8.8   | 8.9                  | 12    | 11                        | 16.4  |
| Osnaburg                     | F                                                             | 9.5   | 10.5                 | 5     | +5*                       | 6.6   |
| Bleached Cotton              | W                                                             | 8.3   | 8.5                  | 17    | 15                        | 12.9  |
| Osnaburg                     | F                                                             | 10.5  | 11.5                 | +5*   | +1.5*                     | 2.3   |
| Wool/PET                     | W                                                             | 9.3   | 9.6                  | 7     | 4                         | 14.4  |
| 65/35                        | F                                                             | 9.2   | 9.7                  | 8     | 3                         | 6.9   |
| Acrylic Tweed                | W                                                             | 9.3   | 9.8                  | 7     | 2                         | 13.5  |
|                              | F                                                             | 9.3   | 9.9                  | 7     | 1                         | 3.0   |
| Acrylic Beige                | W                                                             | 9.3   | 9.9                  | 7     | 1                         | 12.6  |
|                              | F                                                             | 9.4   | 9.9                  | 6     | 1                         | 2.0   |
| PET                          | W                                                             | 9.5   | 9.8                  | 5     | 2                         | 6.0   |
|                              | F                                                             | 9.9   | 10.1                 | 1     | +1                        | 1.0   |

\*+ indicates stretch - only in cotton fabrics

the invention imparts improved surface durability to fabrics without requirement of chemical treatment finishes. This result is obtained through stabilization of fabric matrix structures in the enhancement process through entanglement of yarns. Enhancement simulates fiber locking mechanisms of conventional chemical treatments.

FIGS. 16A,B-18A,B respectively, are macrophotographs of control and processed fabrics as follows: 1) acrylic fabric including wrap spun polyester yarn, 2) 100% polyester fabric including slub yarns, count of 16 x 10 yarns/in<sup>2</sup> and weight of 8 ounces/yd<sup>2</sup>, and 3) Guilford 80% wool/20% nylon fabric (see Table II).

Durability was tested by subjecting the fabric samples to five (5) repeated wash-dry laundering treatments. Test conditions approximated conventional home laundry warm water washing and hot air drying conditions as defined in the AATCC Technical Manual, Test Method 124-1984. Control and process fabrics were mounted on boards and illuminated at an oblique angle by fluorescent light for macrophotographic comparison. Unprocessed fabrics were characterized by a roughened, mottled and nubby finish as compared with enhanced fabrics which exhibit smooth and pressed surface finishes.

**EXAMPLE XV**  
**Shrink-Resistance**

Enhanced fabrics of the invention exhibit enhanced shrink resistance. Tables XII-XIV set forth shrinkage test data for wash/dry and dry cleaning processing of representative control and enhanced fabrics. Fabric shrinkage was measured by marking test fabrics with 10" x 10" measurement lines. Following processing,

TABLE XIII

| Original Sample: 10" x 10" | SHRINKAGE - 5 Dry Cleaning Cycles*<br>WOOL/PET and WOOL/NYLON<br>Warp/Fill (W/F) Measurements |                      |                  |                      |
|----------------------------|-----------------------------------------------------------------------------------------------|----------------------|------------------|----------------------|
|                            | Wool/Pet 65/35                                                                                |                      | Wool/Nylon 80/20 |                      |
|                            | Size<br>(in.)                                                                                 | Percent<br>Shrinkage | Size<br>(in.)    | Percent<br>Shrinkage |
| <u>Control</u>             |                                                                                               |                      |                  |                      |
| W                          | 9.8                                                                                           | 2.0                  | 9.75             | 2.5                  |
| F                          | 9.85                                                                                          | 1.5                  | 9.8              | 2.0                  |
| <u>Processed</u>           |                                                                                               |                      |                  |                      |
| W                          | 9.8                                                                                           | 2.0                  | 9.8              | 2.0                  |
| F                          | 9.85                                                                                          | 1.5                  | 9.9              | 1.0                  |

\*Dry cleaning fluid: Perchloroethylene

TABLE XIV

| 60                      | WOOL SHRINKAGE<br>Samples marked 10" x 10" |       |
|-------------------------|--------------------------------------------|-------|
|                         | Length                                     | Width |
| <u>Fine White Wool</u>  |                                            |       |
| Processed               | 9.75                                       | 9.7   |
| Shrinkage (%)           | 2.5                                        | 3.0   |
| Processed - 5 Wash/Dry  | 8.7                                        | 8.7   |
| Shrinkage (%)           | 13.0                                       | 13.0  |
| Control - 5 Wash/Dry    | 8.3                                        | 8.2   |
| Shrinkage (%)           | 17.0                                       | 18.0  |
| <u>Coarse Blue Wool</u> |                                            |       |
| Processed               | 9.7                                        | 9.3   |
| Shrinkage (%)           | 3.0                                        | 7.0   |
| Processed - 5 Wash/Dry  | 8.0                                        | 8.0   |
| Shrinkage (%)           | 20.0                                       | 20.0  |
| Control - 5 Wash/Dry    | 7.8                                        | 7.7   |

TABLE XIV-continued

| Shrinkage (%) | WOOL SHRINKAGE<br>Samples marked 10" x 10" |       |
|---------------|--------------------------------------------|-------|
|               | Length                                     | Width |
| Shrinkage (%) | 22.0                                       | 23.0  |

## EXAMPLE XVI

## Absorption and Adsorption

Enhanced fabrics of the invention exhibit increased absorption and adsorption properties. Table XV sets forth data for ASTM water retention data for representative fabrics processed in accordance with the invention.

TABLE XV

| Fabric           | Absorptive Capacity<br>Test Standard: ASTM D1117 - 5 sections |         |                  |
|------------------|---------------------------------------------------------------|---------|------------------|
|                  | Untreated                                                     | Treated | Percent Increase |
| Osnaburg         | 11.7                                                          | 12.9    | 10.3             |
| 100% Cotton      |                                                               |         |                  |
| Acrylic          | 16.8                                                          | 21.8    | 29.8             |
| Wool/PET (65/35) | 19.7                                                          | 23.2    | 17.8             |
| PET              | 11.8                                                          | 15.0    | 27.1             |

## EXAMPLE XVII

## Hydromilled Wood

Conventional fulling or felting processes are em-

ployed to finish woolen and worsted fabrics. In such

processes the fabric is subjected to moisture, heat, friction, chemicals and pressure which cause the fabric fibers to mat and densify into a stable structure. Advantageously, it has been found that comparable results are obtained in the present invention without requirement of conventional chemical and mechanical processing and associated degradation of the fabric.

Tables XVI-A-C set forth comparative data for conventional fulled and hydroenhanced griego state wool fabrics. Control and conventional processed fabrics were obtained from Carleton Woolen Mills, Winthrop, Me.. The control griego state fabrics respectively had weights of 180.5, 252.7 and 145.9 gsy prior to application of hydroenhancing and conventional fulling processing. Hydroenhancement data is set forth for processing of each control fabric at energies of 0.5 and 1.0 hp-hr/lb. It will be seen that fabrics processed in accordance with the invention have physical properties which simulate those of the conventionally fulled fabrics.

Wool hydroenhancing ("Hydromilling") trials set forth in Tables XVI-A-C were processed employing the Prototype FIG. 1 line. It is believed that further processing advantage in the hydromilling process could be obtained by use of hot fluid in the entanglement modules. For example, use of hot water in the line will further matting and mechanical entanglement of wool fibers. To this end it would also be advantageous to employ a hot water bath or felting pre-entanglement process step in the invention.

TABLE XVI-A

|                                           | HYDROMILLED WOOL - Sample 1 |            |           |            |
|-------------------------------------------|-----------------------------|------------|-----------|------------|
|                                           | PROCESSED                   |            |           |            |
|                                           | CONTROL*                    | .5 hphr/lb | 1 hphr/lb | FINISHED** |
| WEIGHT (gsy)                              | 180.5                       | 179.6      | 173.9     | 190.9      |
| THICKNESS (mils)                          | 53.2                        | 53.6       | 52.9      | 34.3       |
| AIR PERM (cfm)                            | 329.5                       | 214.0      | 212.0     | 117.4      |
| <u>GRAB TENSILE (lbs)</u>                 |                             |            |           |            |
| WARP                                      | 43.0                        | 43.2       | 41.6      | 35.5       |
| FILL                                      | 31.2                        | 29.4       | 31.7      | 19.1       |
| <u>ELONGATION (%)</u>                     |                             |            |           |            |
| WARP                                      | 42.4                        | 48.5       | 41.1      | 24.5       |
| FILL                                      | 37.5                        | 39.2       | 42.0      | 42.4       |
| <u>TONGUE TEAR (lbs)</u>                  |                             |            |           |            |
| WARP                                      | 6.5                         | 5.2        | 5.4       | 3.0        |
| FILL                                      | 8.3                         | 7.0        | 6.3       | 4.4        |
| <u>% SHRINKAGE<br/>(after 5 wash/dry)</u> |                             |            |           |            |
| WARP                                      | 21.0                        | 17.0       |           | 27.8       |
| FILL                                      | 16.0                        | 17.0       |           | 13.1       |
| TABER ABRASION<br>(% weight loss)         | 4.3                         | 4.0        | 4.1       | 5.0        |
| <u>% WOOL<br/>(Chem. extraction)</u>      | 99.9                        | 100.0      |           |            |

\*Griego state wool, manufactured by Carleton Woolen Mills, Winthrop, Maine.

\*\*Conventional processed wool offered by Carleton Woolen Mills.

ployed to finish woolen and worsted fabrics. In such

TABLE XVI-B

|                           | HYDROMILLED WOOL - Sample 2 |            |           |          |
|---------------------------|-----------------------------|------------|-----------|----------|
|                           | PROCESSED                   |            |           |          |
|                           | CONTROL*                    | .5 hphr/lb | 1 hphr/lb | FINISHED |
| WEIGHT (gsy)              | 252.7                       | 250.8      | 254.7     | 285.5    |
| THICKNESS (mils)          | 69.9                        | 70.8       | 71.4      | 106.6    |
| AIR PERM (cfm)            | 214.5                       | 127.3      | 120.6     | 138.6    |
| <u>GRAB TENSILE (lbs)</u> |                             |            |           |          |
| WARP                      | 52.0                        | 58.9       | 63.8      | 55.1     |
| FILL                      | 53.4                        | 56.5       | 69.5      | 35.9     |
| <u>ELONGATION (%)</u>     |                             |            |           |          |
| WARP                      | 40.0                        | 46.1       | 45.9      | 35.5     |
| FILL                      | 43.2                        | 50.9       | 54.3      | 50.7     |

TABLE XVI-B-continued

| HYDROMILLED WOOL - Sample 2              |           |            |           |          |
|------------------------------------------|-----------|------------|-----------|----------|
|                                          | PROCESSED |            |           |          |
|                                          | CONTROL*  | .5 hphr/lb | 1 hphr/lb | FINISHED |
| <u>TONGUE TEAR (lbs)</u>                 |           |            |           |          |
| WARP                                     | 16.7      | 14.8       | 14.6      | 6.6      |
| FILL                                     | 17.5      | 15.4       | 13.9      | 8.7      |
| <u>% SHRINKAGE</u><br>(after 5 wash/dry) |           |            |           |          |
| WARP                                     | 17.0      | 15.0       | 16.9      |          |
| FILL                                     | 14.0      | 7.0        | 5.6       |          |
| TABER ABRASION                           | 3.7       | 3.6        | 3.0       | 4.4      |
| (% weight loss)                          |           |            |           |          |
| % WOOL                                   | 80.3      | 79.8       |           |          |
| (Chem. extraction)                       |           |            |           |          |

\*Griege state wool manufactured by Carleton Woolen Mills, Winthrop, Maine.

TABLE XVI-C

| HYDROMILLED WOOL - Sample 3              |           |            |           |          |
|------------------------------------------|-----------|------------|-----------|----------|
|                                          | PROCESSED |            |           |          |
|                                          | CONTROL*  | .5 hphr/lb | 1 hphr/lb | FINISHED |
| <u>WEIGHT (gsy)</u>                      |           |            |           |          |
| WARP                                     | 145.9     | 147.7      | 147.3     | 146.9    |
| THICKNESS (mils)                         | 36.6      | 39.7       | 40.5      | 23.2     |
| AIR PERM (cfm)                           | 311.3     | 193.0      | 189.0     | 134.4    |
| <u>GRAB TENSILE (lbs)</u>                |           |            |           |          |
| WARP                                     | 40.7      | 37.7       | 39.5      | 30.4     |
| FILL                                     | 37.3      | 36.5       | 31.8      | 22.9     |
| <u>ELONGATION (%)</u>                    |           |            |           |          |
| WARP                                     | 40.5      | 43.2       | 39.5      | 23.7     |
| FILL                                     | 41.1      | 47.7       | 43.0      | 39.2     |
| <u>TONGUE TEAR (lbs)</u>                 |           |            |           |          |
| WARP                                     | 4.6       | 4.0        | 3.4       | 3.4      |
| FILL                                     | 5.0       | 4.2        | 4.1       | 3.5      |
| <u>% SHRINKAGE</u><br>(after 5 wash/dry) |           |            |           |          |
| WARP                                     | 18.0      | 11.0       | 20.0      |          |
| FILL                                     | 15.0      | 8.0        | 8.1       |          |
| TABER ABRASION                           | 5.0       | 4.5        | 4.7       | 7.2      |
| (% weight loss)                          |           |            |           |          |
| % WOOL                                   | 99.9      | 99.9       |           |          |
| (Chem. extraction)                       |           |            |           |          |

\*Griege state wool manufactured by Carleton Woolen Mills, Winthrop, Maine.

## EXAMPLE XIX

## Flammability

Flame retardancy in conventionally known fabrics is generally obtained by chemical treatment of high melt point fiber based materials. For example, polyester has a melting point in the range of 480°-500° F. and has wide application in the manufacture of flame retardant materials. Such polyester materials are generally subjected to scouring to provide a contaminant free material which in turn is sealed with a chemical finish.

It has been found that polyester fabrics processed in accordance with the invention exhibit increased flame retardancy. Table XVII sets forth flammability test data for plain polyester fabrics samples hydroenhanced in

accordance with the invention. Sample No. 1 designates control and process tests of enhanced fabric which include five (5) specimen trials. Comparative data is set forth for VISA and TREVIRA brand polyester fabrics.

Flame retardancy standards of NFPA are set forth in Table XVIII. The enhanced fabric exhibits flame retardancy properties which exceed those of the VISA and TREVIRA fabrics. It is believed that these results are a function of scouring aspects of the enhancement process as well as the improved stabilization of the fabric matrix obtained by entanglement of yarns. Further advantage in the invention may be obtained by provision of finishes to the fabric to limit introduction of contaminants to the processed fabric.

TABLE XVII

| NFPA 701 - SMALL SCALE<br>POLYESTER FABRICS |          |                    |      |                         |      |                  |
|---------------------------------------------|----------|--------------------|------|-------------------------|------|------------------|
| SAMPLE                                      | SPECIMEN | BURN<br>(12+ sec.) |      | CHAR LENGTH<br>(inches) |      | COMMENTS         |
|                                             |          | warp               | fill | warp                    | fill |                  |
| No. 1C                                      |          | 1                  | 34.6 | 76.4                    | 10.0 | Burns with flame |
|                                             |          | 2                  | 93.7 | 52.6                    | 10.0 |                  |
| CONTROL                                     |          | 3                  | 1.2  | 43.5                    | 5.7  | 10.0             |
| 5.5 osy                                     |          | 4                  | 32.0 | 13.4                    | 10.0 | Some drips       |
|                                             |          | 5                  | 47.0 | 27.6                    | 10.0 | (1-13 sec.)      |
| AVG. - 5 specimens                          |          |                    |      | 41.7                    | 42.7 | 9.1              |
| 10 specimens                                |          |                    |      |                         |      | 9.3              |
| No. 1P                                      |          | 1                  | 3.9  | 0                       | 4.0  | 4.5              |
|                                             |          |                    |      |                         |      | Melts and        |

TABLE XVII-continued

| SAMPLE                             | SPECIMEN | BURN<br>(12+ sec.) |      | CHAR LENGTH<br>(inches) |                    | COMMENTS     |
|------------------------------------|----------|--------------------|------|-------------------------|--------------------|--------------|
|                                    |          | warp               | fill | warp                    | fill               |              |
| HYDROENHANCED<br>5.4 osy           | 2        | 0                  | 0    | 5.0                     | 3.8                | shrinks from |
|                                    | 3        | 10.1               | 23.1 | 4.2                     | 4.0                | flame        |
|                                    | 4        | 0                  | 0    | 3.6                     | 3.8                | Few drips    |
|                                    | 5        | 0                  | 0    | 5.3                     | 3.0<br>(1 sec.)    |              |
| AVG. - 5 specimens<br>10 specimens |          | 2.8                | 4.6  | 4.4                     | 3.8                |              |
|                                    |          |                    |      | 4.1                     |                    |              |
| No. 2                              | 1        | 0                  | 0    | 4.3                     | 4.1                | Melts and    |
|                                    | 2        | 0                  | 0    | 3.5                     | 5.3                | shrinks      |
| VISA*                              | 3        | 0                  | 0    | 4.3                     | 6.0                | from flame   |
| FR treated                         | 4        | 0                  | 0    | 4.1                     | 5.8                |              |
| 4.8 osy                            | 5        | 0                  | 0    | 5.6                     | 4.6                |              |
| AVG. - 5 specimens<br>10 specimens |          | 0                  | 0    | 4.4                     | 5.2                |              |
|                                    |          |                    |      | 4.2                     |                    |              |
| No. 3                              | 1        | 3.8                | 10.7 | 4.0                     | 4.9                | Burns with   |
|                                    | 2        | 0                  | 6.8  | 4.8                     | 4.8                | flame        |
| TREVIRA**                          | 3        | 0                  | 5.2  | 6.0                     | 4.2                |              |
| Inherently FR                      | 4        | 0                  | 1.8  | 5.8                     | 4.6                | Some drips   |
| 4.2 osy                            | 5        | 0                  | 2.1  | 4.9                     | 5.2<br>(1-13 sec.) |              |
| AVG. - 5 specimens<br>10 specimens |          | 0.8                | 5.3  | 5.1                     | 4.7                |              |
|                                    |          |                    |      | 5.1                     |                    |              |

\*VISA is a trademark of Milliken Research Corporation, Spartanburg, South Carolina.

\*\*TREVIRA is a trademark of Hoechst Celanese Corporation, Charlotte, North Carolina.

The following table from NFPA 701 sets forth the allowable limits for these fabrics.

TABLE XVIII

| Permissible Length of Char or Destroyed<br>Material - Small Scale Test |                                                |                                                     |
|------------------------------------------------------------------------|------------------------------------------------|-----------------------------------------------------|
| Weight of Material<br>Being Tested<br>(oz per sq. yd.)                 | Maximum Average<br>of 10 Specimens<br>(inches) | Maximum Individual<br>for Each Specimen<br>(inches) |
| Over 10                                                                | 3.5                                            | 4.5                                                 |
| Over 6 and not<br>exceeding 10                                         | 4.5                                            | 5.5                                                 |
| Not exceeding 6                                                        | 5.5                                            | 6.5                                                 |

FIG. 19 illustrates an alternative embodiment of the invention apparatus, generally designated 40. The apparatus includes a plurality of drums 42a-d over which a fabric 44 is advanced for enhancement processing. Specifically, the fabric 44 traverses the line in a sinuous path under and over the drums 42 in succession. Rollers 46a and b are provided at opposite ends of the line adjacent drums 42a and d to support the fabric. Any or all of the drums can be rotated by a suitable motor drive (not shown) to advance the fabric on the line.

A plurality of manifolds 48 are provided in groups, FIG. 19 illustrates groups of four, which are respectively spaced from each of the drums 42a-d. An arrangement of manifold groups at 90° intervals on the sinuous fabric path successively positions the manifolds in spaced relation with respect to opposing surfaces of the fabric. Each manifold 48 impinges columnar fluid jets 50, such as water, against the fabric. Fluid supply 52 supplies fluid to the manifolds 48 which is collected in liquid sump 54 during processing for recirculation via line 56 to the manifolds.

The support drums 42 may be porous or non-porous. It will be recognized that advantage is obtained through use of drums which include perforated support surfaces. Open areas in the support surfaces facilitate recirculation of the fluid employed in the enhancement process.

Further advantage is obtained, as previously set forth in discussion of the first embodiment, through use of support surfaces having a fine mesh open area pattern which facilitates fluid passage. Offset arrangement of

the support member orientations, for example at 45° offset orientation as shown in FIG. 2, limits process water streak and weave reed marks in the enhanced fabric.

Enhancement is a function of energy which is imparted to the fabric. Preferred energy levels for enhancement in accordance with the invention are in the range of 0.1 to 2.0 hp-hr/lb. Variables which determine process energy levels include line speed, the amount and velocity of liquid which impinges on the fabric, and fabric weight and characteristics.

Fluid velocity and pressure are determined in part by the characteristics of the fluid orifices, for example, columnar versus fan jet configuration, and arrangement and spacing from the process line. It is a feature of the invention to impinge a curtain of fluid on a process line to impart an energy flux of approximately 0.46 hp-hr/lb to the fabric. Preferred specifications for orifice type and arrangement are set forth in description of the embodiment of FIG. 1. Briefly, orifices 16 are closely spaced with center-to-center spacings of approximately 0.017 inches and are spaced 0.5 inches from the support members. Orifice diameters of 0.005 inches and densities of 60 per manifold inch eject columnar fluid jets which form a uniform fluid curtain.

The following Examples are representative of the results obtained on the process line illustrated in FIG. 20.

#### EXAMPLE XX

A plain woven 100% polyester fabric comprised of friction spun yarns having the following specifications was processed in accordance with the invention: count of 16×10 yarns/in<sup>2</sup>, weight of 8 ounces/yd<sup>2</sup>, an abrasion resistance of 50 cycles (measured by 500 grams of a CS17 abrasion test wheel) and an air permeability of 465 ft<sup>3</sup>/ft<sup>2</sup>/min.

The fabric was processed on a test line to simulate a speed of 300 ft/min. on process apparatus including four drums 42 and eighteen nozzles 16 at a pressure of approximately 1500 psi. Energy output to fabric at these process parameters was approximately 0.46 hp-hr/lb.

Table XIX sets forth control and processed characteristics of the fabric.

TABLE XIX

| 100% Polyester Friction Spun' Fabric                     |         |           |
|----------------------------------------------------------|---------|-----------|
| Fabric Characteristic                                    | Control | Processed |
| Count (yarns/in. <sup>2</sup> )                          | 16 x 10 | 17 x 10   |
| Weight (ounces/yd. <sup>2</sup> )                        | 8       | 8.2       |
| Abrasion resistance (cycles)                             | 50      | 85        |
| Air permeability (ft <sup>3</sup> ft <sup>2</sup> /min.) | 465     | 181       |

## EXAMPLES XXI AND XXII

The process conditions of Example XX were employed to process a plain woven cotton osnaburg and plain woven polyester ring spun fabrics yielding the results set forth in Tables XX and XXI.

TABLE XX

| Plain Woven Cotton Osnaburg                              |         |           |
|----------------------------------------------------------|---------|-----------|
| Fabric Characteristic                                    | Control | Processed |
| Count (yarns/in. <sup>2</sup> )                          | 32 x 26 | 32 x 32   |
| Abrasion resistance (cycles)                             | 140     | 344       |
| Air permeability (ft <sup>3</sup> ft <sup>2</sup> /min.) | 710     | 120       |

TABLE XXI

| Plain Woven Polyester Ring Spun Yarn                     |         |           |
|----------------------------------------------------------|---------|-----------|
| Fabric Characteristic                                    | Control | Processed |
| Count (yarns/in. <sup>2</sup> )                          | 44 x 28 | 48 x 32   |
| Abrasion resistance (cycles)                             | 100     | 225       |
| Air permeability (ft <sup>3</sup> ft <sup>2</sup> /min.) | 252     | 63        |

Fabrics processed in Examples XX-XXI are characterized by a substantial reduction in air permeability and increase in abrasion resistance. Process energy levels in these Examples were approximately 0.46 hp-hr/lb. It has been discovered that there is a correlation between process energy and enhancement. Increased energy levels yield optimum enhancement effects.

The foregoing Examples illustrate applications of the hydroenhancing process of the invention for upgrading the quality and physical properties of single ply woven and knit fabrics.

In an alternative application of the hydroenhancing process of the invention, fabric strata are hydrobonded into integral composite fabric. FIG. 20 illustrates a composite flannel fabric 60 including fabric layers 62, 64. Hydrobonding of the layers is effected by first napping opposing surfaces 62a, 64a of each of the layers to raise surface fibers. The opposing surfaces 62a, 64a are then arranged in overlying relation and processed on the production line of the invention. See FIGS. 1 and 16. Enhancement of the layers 62, 64 effects entanglement of fibers in the napped surfaces and bonding of the layers to form a integral composite fabric 60. Exterior surfaces 62b, 64b are also enhanced in the process yielding improvements in cover and quality in the composite fabric.

Napped surfaces 62a, 62b are provided by use of conventional mechanical napping apparatus. Such apparatus include cylinders covered with metal points or teasel burrs which abrade fabric surfaces.

Advantageously, composite fabric 60 is manufactured without requirement of conventional laminating adhesives. As a result, the composite fabric breaths and has improved tactile characteristics than obtained in prior art laminated composites. It will be recognized that

such composite fabrics have diverse applications in fields such as apparel and footwear.

Advantageous results may also be obtained by hydro-enhancing a single strata napped fabric. Entanglement of raised fibers in a napped fabric surface obtained in the invention process yield a superior fabric finish.

FIGS. 21A and B illustrate a composite nonwoven-woven composite fabric in accordance with a further embodiment of the invention. The fabric composite 70 includes a carded nonwoven and woven layers 72, 74 which are arranged in opposing relation and hydrobonded employing enhancement processing. Hydrobonding of the layers and entanglement of the carded nonwoven layer 72 is effected in a one step fluid treatment process. Enhancement of the bonded composite yields a fabric having improved cover and finish. Such nonwoven-woven composite materials have application, among others, for use as interliner materials in textile products.

In another embodiment of the invention, woven or knit fabrics are provided which comprise wrap spun yarns having a fibrous sliver core and water soluble outer sheath components. Enhancement processing effects wash-out of the soluble sheath and entanglement of sliver core fibrous material to yield a stabilized fabric. Wrap spun yarns impart structural integrity to the fabric useful to facilitate weaving of yarns into a stable material for enhancement processing. Enhancement of the fabric and wash-out of the wrap yields a delicate fabric of superior structural integrity. In a preferred application the fabric yarns include a cotton fiber sliver core having a PVA filament wrap, and both top and bottom surfaces of the fabric are subjected to hydraulic enhancement.

Optimum enhancement (in single and multi-ply fabrics) is a function of energy. Preferred results are obtained at energy levels of approximately 0.5 hp-hr/lb. Energy requirements will of course vary for different fabrics as will process conditions required to achieve optimum energy levels. In general, process speeds, nozzle configuration and spacing may be varied to obtain preferred process energy levels.

Enhanced fabrics of the invention are preferably fabricated of yarns including fibers having deniers and lengths, respectively, in the ranges of 0.3 to 10.0 and 0.5 to 6.0 inches, and yarn counts of 0.5 s to 80 s. Optimum enhancement is obtained in fabrics having fiber deniers in the range of 0.5 to 6, staple fibers of 0.5 to 6.0 inches, and yarn counts in the range of 0.5 s to 50 s. Preferred yarn spinning systems employed in the invention fabrics include cotton spun, wrap spun and wool spun. Experimentation indicates that preferred enhancement results are obtained in fabrics including low denier, short lengths fibers, and loosely twisted yarns.

The invention advances the art by recognizing that superior fabric enhancement can be obtained under controlled process conditions and energy levels. Heretofore, the art has not recognized the advantages and the extent to which hydroenhancement can be employed to upgrade fabric quality. It is submitted that the results achieved in the invention reflect a substantial and surprising contribution to the art.

Numerous modifications are possible in light of the above disclosure. For example, although the preferred process and apparatus employ fluid pervious support members, non-porous support members are within the scope of the invention. Similarly, FIGS. 1 and 20 respectively illustrate two and four stage enhancement

process lines. System configurations which include one or more modules having flat, drum or other support member configuration may be employed in the invention.

It will be recognized that the process of the invention has wide application for the production of a diversity of enhanced fabrics. Thus, the Examples are not intended to limit the invention.

Finally, although the disclosed enhancement process employs columnar jet orifices to provide a fluid curtain, other apparatus may be employed for this purpose. Attention is directed to the U.S. Pat. No. 4,995,151 to Siegel et al., entitled "Apparatus and Method For Hydropatterning Fabric", dated Feb. 26, 1991, assigned to International Paper Company, assignee of the present case, which discloses a divergent jet fluid entangling apparatus for use in hydropatterning woven and non-woven textile fabrics.

Therefore, although the invention has been described with reference to certain preferred embodiments, it will be appreciated that other hydroentangling apparatus and processes may be devised, which are nevertheless within the scope and spirit of the invention as defined in the claims appended hereto.

We claim:

1. An enhanced woven or knit textile fabric which comprises: spun and/or spun filament yarns which intersect at cross-over points to define interstitial open areas and a fabric matrix, said yarns being treated with high pressure fluid energy to effect entanglement thereof in said interstitial open areas, wherein said fluid treatment effects stabilization of said fabric matrix, such that the enhanced woven or knit textile fabric exhibits improved shrink resistance, surface durability, and material absorption and adsorption characteristics.

2. An enhanced woven or knit textile fabric according to claim 1, wherein the fabric includes wool fibers, and the stabilization provides a fabric which is shrink resistant and washable.

3. An enhanced woven or knit textile fabric according to claim 2, wherein the fabric further comprises a second textile fiber.

4. An enhanced woven or knit textile fabric according to claim 3, wherein said textile fiber is polyester.

5. An enhanced woven or knit textile fabric according to claim 1, wherein said fabric includes polyester, and said fluid treatment imparts flame resistance to the fabric.

6. An enhanced woven or knit textile fabric according to claim 1, wherein the fabric includes a napped surface finish having raised surface fibers, said napped finish being subjected to said fluid treatment said fluid treatment entangling said raised fibers and providing a fabric having improved structural integrity and a high 55 loft finish.

7. An enhanced woven or knit textile fabric according to claim 1, wherein the fabric includes wrap spun yarn, said yarn having a sliver core of a first fibrous component, and an outer sheath wrap of a water soluble 60 yarn, said wrap yarn imparting structural integrity to the fabric for textile weaving or knit fabrication, said fluid treatment effecting wash-out of said soluble sheath to provide a stabilized fabric of said first fibrous component having structural integrity.

8. An enhanced woven or knit textile fabric according to claim 7, wherein said sliver core includes cotton fibers, and said outer sheath wrap includes filament

fibers selected from the group consisting of polyester and nylon.

9. An enhanced woven or knit textile fabric according to claim 1, wherein said fabric includes wool fibers, a felt and matted finish is imparted to the fabric by hot water treatment, and said fluid entanglement treatment effects interlocking and stabilization of said wool fibers.

10. An enhanced woven or knit textile fabric according to claim 9, wherein said fabric further comprises a 10 second textile fiber.

11. An enhanced woven or knit textile and nonwoven fabric composite comprising: a fabric layer which includes spun and/or spun filament yarns in a structured pattern of yarns which intersect at cross-over points to 15 define interstitial open areas, and a nonwoven layer which includes staple fibers, said fabric and nonwoven layers being arranged in opposing and congruent relation and bonded into an integral composite by treatment with high-pressure fluid energy, wherein said spun and/or spun filament yarns are entangled within said interstitial open areas and said spun and/or spun filament 20 yarns are also entangled with said staple fibers.

12. An enhanced composite fabric according to claim 11, wherein said nonwoven layer comprises a carded 25 web of staple fibers.

13. A method for hydrobonding woven or knit fabric and nonwoven material layers to form a composite textile fabric, the fabric layer including spun and/or spun filament yarns in a structured pattern which intersect at crossover points to define interstitial open areas, the nonwoven layer including staple fibers, the method comprising the steps of:

arranging said fabric and nonwoven layers in opposing and overlying layered relation,  
35 supporting the layered fabric on a support member, and  
traversing one side of said layered fabric with a first continuous curtain of fluid for sufficient duration to entangle said spun and/or spun filament yarns in said interstitial open areas and also entangle said staple fibers and spun and/or spun filament yarns, said curtain of fluid impacting the fabric with an energy in the range 0.1 and 2.0 hp-hr/lb.

14. The method of claim 13, wherein said fluid curtain is provided by columnar fluid jet orifices having a diameter of approximately 0.005 inches and center-to-center spacing of approximately 0.017 inches, said fluid curtain impinging the fabric with fluids at a pressure of approximately 1500 psi.

15. The method of claim 14, wherein said support member includes a pattern of closely spaced fluid pervious open areas aligned in a first direction to effect fluid passage through said support member.

16. The method of claim 14, comprising the further steps of:

supporting said layered fabric on a second support member, and  
traversing the other side of said layered fabric in a second entanglement stage with a second continuous fluid curtain to effect a uniform composite fabric bond and finish,  
said second entanglement stage impacting the layered fabric with an energy in the range 0.1 and 2.0 hp-hr/lb.

17. The method of claim 16, wherein:  
said first and second fluid curtains are provided by columnar fluid jets having a diameter of approximately 0.005 inches and center-to-center spacing of

approximately 0.017 inches, said fluid jets impinging the fabric with fluids at pressure of approximately 1500 psi, said first and second support members each include a pattern of closely spaced fluid pervious open areas, respectively aligned in first and second directions, said open areas being dimensioned to effect fluid passage through said support members without imparting a patterned effect to the fabric.

18. A method for enhancing and finishing textile fabrics including spun wool yarns in a structured woven or knit pattern including yarns which intersect at cross-over points, the method comprising the steps of:

felting the fabric by application of hot water treatments to form a matted and integrated fabric finish, supporting the fabric on a first support member, and traversing a first side of said fabric with a first continuous curtain of fluid for sufficient duration to effect entanglement of said yarns at the cross-over points, thereby enhancing fabric cover and quality, said curtain of fluid impacting the fabric with an energy in the range 0.1 and 2.0 hp-hr/lb.

19. The method of claim 18, wherein said fluid curtain comprises hot water.

20. The method of claim 18, wherein said fluid curtain is provided by columnar fluid jet orifices having a diameter of approximately 0.005 inches, center-to-center spacing of approximate 0.017 inches, and spacing from said first support member of approximately 0.5 inches, said fluid jets impinging the fabric with fluids at a pressure of approximately 1500 psi.

21. The method of claim 20, wherein said support member includes a pattern of closely spaced fluid pervious open areas aligned in a first direction to effect fluid passage through said support member.

22. The method of claim 19, comprising the further steps of:

supporting said enhanced fabric on a second support member, and traversing a second side of said enhanced fabric in a second enhancement stage with a second continuous fluid curtain for sufficient duration to further

enhance fabric cover and provide a uniform fabric finish, said second enhancement stage impacting the fabric with an energy in the range 0.1 and 2.0 hp-hr/lb.

23. A method for enhancing and finishing textile fabrics including wrap spun yarns in a structured woven or knit pattern which intersect at cross-over points, the fabric including a sliver core of a first fibrous component, and an outer sheath wrap of a water soluble yarn, the method comprising the steps of:

supporting the fabric on a first support member, and traversing a first side of said fabric with a first continuous curtain of fluid for sufficient duration to effect wash-out of the soluble wrap and entanglement of said yarns at the cross-over points, thereby providing a stabilized core material fabric having integrity and enhanced finish, said curtain of fluid impacting the fabric with an energy in the range 0.1 and 2.0 hp-hr/lb.

24. The method of claim 23, wherein said fluid curtain is provided by columnar fluid jet orifices having a diameter of approximately 0.005 inches, center-to-center spacing of approximately 0.17 inches, and spacing from said first support member of approximately 0.5 inches, said fluid jets impinging the fabric with fluids at pressure of approximately 1500 psi.

25. The method of claim 24, wherein said support member includes a pattern of closely spaced fluid pervious open areas aligned in a first direction to effect fluid passage through said support member.

26. The method of claim 25, comprising the further steps of:

supporting said enhanced fabric on a second support member, and traversing a second side of said enhanced fabric in a second enhancement stage with a second continuous fluid curtain for sufficient duration to further enhance fabric cover and provide a uniform fabric finish,

said second enhancement stage impacting the fabric with an energy in the range 0.1 and 2.0 hp-hr/lb.

\* \* \* \* \*